

3,082,110  
STABILIZED YARN

Robert C. Harrington, Jr., and James L. Smith, Kingsport, Tenn., assignors to Eastman Kodak Company, Rochester, N.Y., a corporation of New Jersey  
No Drawing. Filed Oct. 25, 1960, Ser. No. 64,694  
7 Claims. (Cl. 106—194)

This invention relates to a composition of matter, especially a cellulose ester containing composition which composition exhibits stability to actinic radiation. More particularly, this invention relates to dull and semi-dull cellulose ester filaments which are relatively highly stable toward photodegradation.

It is already well known in the industry to prepare spinning solutions of spinnable materials such as cellulose esters dissolved in a solvent. It is further known to extrude such spinning solutions through spinnerettes to form filaments therefrom by the elimination of the solvent from the extruded materials. In the manufacture of the so-called dull or semi-dull or delustered fibers, it is customary to include a pigment in the spinning solution for obtaining the dull or delustered effect. As is well known, titanium dioxide in finely divided form is a frequently used delustering pigment.

Studies have shown that scission of the polymer chain of the fiber forming material by light is catalyzed by titanium dioxide. Therefore, photodegradation of dull or semi-dull or the like delustered fibers is more severe than for the so-called bright yarns which do not include or include a lesser amount of such pigments as titanium dioxide. In order to retard such type photodegradation especially in the dull or delustered fibers as just referred to, it has already been proposed to incorporate ultraviolet light absorbing materials and antioxidants into the spinning compositions or onto the surface of the fibers or fabrics woven therefrom. Presumably the functioning of prior additives has been postulated on the theory that peroxides are formed in the fibers through the absorption of ultraviolet radiations. Thus the fiber material might be protected if the rays or radiation can be absorbed preferentially by some compound incorporated in the fiber or if the peroxides once formed are quickly taken care of by some agent such as an antioxidant in the fiber.

While prior art methods of stabilization have received some favorable acceptance in the industry, it is apparent that the development of further more simplified or different procedures for stabilizing cellulose ester compositions represents a highly desirable result. After extended investigation we have found a procedure of stabilizing and a stabilizing agent which appears not only to very efficiently function, but to function by a mechanism different from the prior art stabilizers and in a manner, the principle of which is presently unknown to us.

This invention has for one object to provide compositions of matter especially compositions containing a substantial content of cellulose acetate which compositions exhibit relatively good stability toward actinic radiations. A particular object is to provide a cellulose acetate spinning solution which is relatively highly stable to actinic radiation and which may be spun into filaments wherein the resultant filaments not only possess their original properties, but have better stability to photodegradation. A further object is to provide cellulose acetate fibers so stabilized that they are not substantially deleteriously affected with respect to strength, elongation or color. A still further object is to provide procedure for incorporating certain novel additives into cellulose ester spinning solutions and the spinning of fibers from such solutions. Other objects will appear hereinafter.

In the broader aspects of the present invention we

have found that compositions of matter and more particularly exemplified by spinning solutions which may have added thereto a small portion of zinc acetyl acetate with the beneficial effect that such combination and the extruded products resulting therefrom have decreased rate of photodegradation. Zinc acetyl acetate is a compound having the following type formula



In general we have found that a concentration as low as 0.1% based on the weight of the composition of matter will give a beneficial effect. Usually we would not use more than 1.5% by weight. In the instance of cellulose ester spinning solutions we have found that a concentration between 0.4% and 0.7% based on the cellulose ester weight is quite satisfactory. We have found that our zinc acetyl acetate additive is particularly effective in cellulose ester spinning solutions which contain titanium dioxide delustering or dulling agents.

In further detail, zinc acetyl acetate may be prepared by the following procedure. Four hundred ml. of absolute ethyl alcohol were placed in a flask fitted with stirrer, condenser and thermometer. The alcohol was protected from atmospheric moisture by means of a calcium chloride tube. One mole, 23 grams, of sodium was added in small pieces. After all the sodium had reacted, one mole of 2,4-pentanedione (acetyl acetone) was slowly added. The solution was maintained for 30 minutes at a temperature sufficient to cause refluxing. Then 1/2 mole (68.2 grams) of anhydrous zinc chloride dissolved in absolute alcohol was added over a 20-minute period and the mixture was maintained at refluxing temperature for an hour. The mixture was filtered while hot to remove precipitated sodium chloride. Zinc acetyl acetate crystallized from the filtrate on cooling. It was collected by filtration and recrystallized from ethyl alcohol.

While we prefer the foregoing type of method for producing the zinc acetyl acetate, the exact source of the additive or its method of manufacture is not a limitation on the present invention. A suitable quality zinc acetyl acetate is obtained and then ground in the presence of the type of solvent that is to be used in dissolving the solid material from which the fibers are to be produced. For example, in the instance of cellulose acetate, acetone is the type of solvent usually used for dissolving the cellulose acetate. Therefore, the zinc acetyl acetate would be ground in the presence of acetone. A spinning solution may be made in the usual way from the filament forming material, titanium dioxide or comparable delusterant, coloring material or the like together with 0.1% to 1.5% of the zinc acetyl acetate of the present invention. Such spinning solutions may then be spun into filaments by conventional procedures such as dry spinning, wet spinning, melt spinning or the like to produce filaments which exhibit greater resistance to actinic radiation either in the filament form or in the form of products such as fabrics.

A further understanding of our invention may be had from a consideration of the following examples which are set forth for illustrating certain preferred embodiments.

*Example I*

In accordance with this example the white fine acetyl acetate powder-like solid was ground in the presence of acetone. This mixture was added to a 27% solution of secondary cellulose acetate in acetone in which 1.4% based on the acetate weight, of titanium dioxide had been suspended. The concentration of zinc acetyl acetate was 0.5% based on the weight of cellulose acetate.

late. The solution was dry spun in a conventional manner by extruding it through small orifices into a drying chamber to remove the solvent. Continuous filament yarn of 150 denier with 38 filaments prepared as described above was used as filling in a 75-denier bright acetate warp. A satin weave was used wherein the yarn showing on the dull side of the fabric commonly referred to as the back, was about 80% cellulose acetate containing 0.5% zinc acetyl acetone. The fabric was exposed to light rich in ultraviolet in a Fade-Ometer, an instrument utilizing a carbon arc. The dull side of the fabric was turned toward the light. A control fabric, identical to the one described above except that the 150 denier full yarn contained no zinc acetyl acetone, was exposed to light in the same manner.

Strips of each fabric were exposed in a Fade-Ometer for 400 and 600 hours. Before exposure and after each time period the samples were tested. The forces were measured which were necessary to pull apart, in a longitudinal direction, strips one inch wide and three inches long. The strips had been cut from the fabric samples so that the filling was running longitudinally and thus the pulling was done against the fibers in the filling. The fibers containing zinc acetyl acetone retained a much larger portion of their original strength and lost strength less quickly than the control samples. After 400 hours the control sample had lost 57% of its original strength while the one containing zinc acetyl acetone had lost 32%. After 600 hours, the sample containing the zinc compound was 62% stronger than the control.

#### Example II

Yarn containing 0.1% zinc acetyl acetone was prepared and tested in an analogous manner to the yarn in Example I. After 600 hours in a Fade-Ometer the fabric was 38% stronger than a control fabric.

#### Example III

A fiber forming spinning solution consisting of acetone solvent, cellulose acetate (39.3% acetyl) at a concentration of 27%, and zinc acetyl acetone at a concentration of 0.5% based upon the acetate weight was dry spun in a conventional manner. The fibers of 4 denier per filament were wound on wire frames and exposed in a Fade-Ometer for 400 hours. Control fibers containing no zinc acetyl acetone were prepared and tested in the same manner. The stabilized fibers lost only 7.1% of their strength while the control fibers lost 29%. In other words the stabilized fibers were losing strength at only 1/4 the rate of the control fibers. After the same exposure period, the percent loss in the elongation of the control fibers was 60 while the stabilized fiber lost only 0.55 percent of its original elongation. It should be noted, as illustrated by this example, that zinc acetyl acetone also serves as a stabilizer in the absence of titanium dioxide.

#### Example IV

Two films of cellulose acetate butyrate, 13% acetyl and 37% butyryl, one containing 0.7% zinc acetyl acetone and the other no stabilizer were cast from acetone solutions. The films, 0.05 inch thick were exposed to ultraviolet light in a Fade-Ometer for 400 hours. The intrinsic viscosities of the polymers were determined both before and after exposure. The stabilized polymer lost only 2 percent of its original intrinsic viscosity while the control which contained no zinc acetyl acetone lost 18 percent. Loss in intrinsic viscosity is indicative of a corresponding loss in strength.

#### Example V

Example IV was repeated except that cellulose triacetate films, one with 0.7% zinc acetylacetone and the other without the stabilizer, were cast from a solvent consisting of nine parts of methylene chloride and one part of

methanol by weight. After 400 hours in the Fade-Ometer the stabilized film had lost 6% of its original intrinsic viscosity while the control had lost 20%.

It can be seen from the foregoing description that we have provided a number of new compositions of matter, particularly in the form of spinning solutions.

Such spinning solutions enable the production of filamentary and fabric products that are more resistant to actinic radiation than comparable products heretofore available. While our invention is particularly applicable to cellulose acetate compositions in the form of acetone spinning solutions made therefrom, certain other benefits of our invention may be had in combination with other types of fiber and film forming materials. Illustrations of these variations are as follows: cellulose triacetate, cellulose tripropionate, cellulose acetate butyrate and mixtures of cellulosic esters with other polymers.

Although we prefer to use acetone as the solvent for the fiber forming materials and for grinding the additive, since it is a well-known readily available commercial solvent, other solvents and solvent combinations may be used illustrated by the following: chlorinated hydrocarbons such as methylene chloride and tetrachloroethane, chlorinated hydrocarbons mixed with low molecular weight alcohols such as that illustrated in Example V, and lower N,N dialkyl alkanamides such as dimethyl formamide.

The invention has been described in detail with particular reference to preferred embodiments thereof, but it will be understood that variations and modifications can be effected within the spirit and scope of the invention as described hereinabove and as defined in the appended claims.

We claim:

1. As a new composition of matter adapted for spinning, a solution consisting principally of a lower cellulose ester, a solvent for said lower cellulose ester, and 0.1 to 1.5% of zinc acetyl acetone based on the weight of said lower cellulose ester.
2. A composition according to claim 1 wherein the cellulose ester consists essentially of cellulose acetate and 0.25 to 5% by weight of said cellulose ester of titanium dioxide.
3. As a new article of manufacture, a fabric comprising a lower cellulose ester, 0.1 to 1.5% zinc acetyl acetone based on the weight of said lower cellulose ester, and 0.2 to 5% titanium dioxide based on the weight of said lower cellulose ester.
4. A product in accordance with claim 3 wherein the lower cellulose ester consists essentially of cellulose acetate.
5. As a new article of manufacture, a fabric which consists essentially of lower cellulose ester fibers containing 0.1 to 1.5% by weight of zinc acetyl acetone whereby the fibers exhibit enhanced resistance to photodegradation.
6. A product in accordance with claim 5 wherein the lower cellulose ester consists essentially of cellulose acetate.
7. The method of preparing filaments of increased resistance to actinic radiation which comprises dry spinning a solution of cellulose acetate, 0.1 to 1.5% zinc acetyl acetone based on the weight of said cellulose acetate and 0.25 to 5% titanium dioxide based on the weight of said cellulose acetate.

#### References Cited in the file of this patent

#### UNITED STATES PATENTS

- 70 2,615,860 Burgess ----- Oct. 28, 1952  
2,819,978 Long et al. ----- Jan. 14, 1958

#### FOREIGN PATENTS

- 830,475 France ----- Aug. 1, 1938